

## UNITED STATES PATENT OFFICE

1,920,559

THERMOELECTRIC ELEMENT AND  
THERMOCOUPLEOtto Hermann, St. Louis, Mo., assignor to  
Thermo Electric Company, St. Louis, Mo., a  
Corporation of MissouriNo Drawing. Application July 30, 1931  
Serial No. 554,166

2 Claims. (Cl. 136—5)

My invention relates to a thermo-couple and more particularly to a thermo-electric member therefor consisting of an alloy containing three metallic elements. The principal object of the 5 invention is a thermo-couple adapted to produce a larger quantity of electrical energy for a given quantity of heat absorbed at the hot junction of the thermo-couple than has been produced by prior thermo-couples. Other objects of the 10 invention are a thermo-couple which can be cheaply produced and a thermo-electric member especially adapted for use as the negative member of a thermo-couple.

My invention consists principally in a thermo-electric member composed of an alloy of antimony, arsenic and zinc, antimony being the base metal. The invention further consists in the thermo-electric member and thermo-couple hereinafter described and claimed.

20 The negative thermo-electric member embodying my invention is an alloy composed of antimony, arsenic and zinc, the preferred range of ingredients being from 60 to 63% antimony, 34 to 37% zinc and 1 to 4.5% arsenic. Typical compositions are: 60.7% antimony, 36.3% zinc, 3% arsenic; 62.7% antimony, 36.3% zinc, 1% arsenic.

Said alloy has been found to be highly negative against all commercial metals and alloys, including silver, alloys of silver and nickel and 30 alloys of copper and nickel. A thermo-couple having this alloy as the negative member and an alloy containing 55% copper and 45% nickel as the positive member produces an electro-motive force of .09 volt at a difference in temperature 35 between the junctions as low as 300° C.

According to the preferred process of making said negative alloy metal, the antimony is melted and heated to a temperature from 70 to 100° above its melting point and the arsenic is added 40 thereto. The arsenic is quickly dissolved in the melted antimony without any appreciable loss of the arsenic by evaporation. The zinc is then added to the arsenic-antimony mixture and readily alloys therewith.

45 The alloy is very hard and is strong enough in cast form for use in thermocouples. The melting point of the alloy is around 650° C. when it contains 4% arsenic. The alloy resists oxidation at elevated temperatures up to 380° 50 C. or higher.

In addition to the properties already mentioned said negative alloy has a low thermal conductivity and an electrical conductance compared therewith high enough to permit flow of a relatively large current. Since the ratio of the two

conductivities, electrical and thermal, in both members (especially in the negative member) is not equal to unity, the electrical conductance in both members being smaller than the thermal conductance, the difference in their sizes with 60 respect to their cross sectional areas can not correspond simply to the ratio of their electrical conductance, but the cross sectional areas of the two elements must bear a quantitative relation to one another based on both the electrical and thermal conductance. Other conditions being equal, the maximum electrical efficiency of a thermocouple is obtained when the ratio of the cross sectional areas of the two members of the thermo-couple equals 65

$$\sqrt{\frac{sI}{s'I'}}$$

where  $s$  and  $I$  denote the two conductivities of one member and  $s'$  and  $I'$  those of the other member. It has been proved by experiment that when the sizes of the members with respect to their cross sectional areas are determined by the above ratio, the electrical conductance of the thermo-couple and the flow of current in the same approach a maximum, while the heat carried off by conduction from the hot to the cold junction is at a minimum. The ratio of the cross sectional area of the positive element, when composed of 55% copper and 45% nickel, to the cross 80 sectional area of the negative member is about 1 to 48 or more depending greatly upon the relative quantities of the component metallic elements contained in the negative alloy metal. The arsenic, in particular, is an important factor. 85

In view of the great differences between the physical properties of the alloy material and those of the positive material, the process of uniting the members of the thermo-couple is 90 of prime importance. According to my preferred process, the negative alloy material is cast around the end portion of the positive member, said positive member having the form of a wire or ribbon. If the positive member is composed of silver or of silver alloy, the negative material 95 may be cast directly thereon. When the positive member is composed of other material, such as the hereinbefore mentioned alloy of 55% copper and 45% nickel, one or both ends of the positive thermo-couple member must be covered with a film of silver, after which the molten negative alloy material may be cast around the positive member. It has been found by experiment 100 that the negative alloy metal makes a firm and persistent contact with said layer of silver or 105

110

with an alloy containing silver. Without the presence of silver in the positive member, or as a coating thereon, the negative member can not be made to make proper contact therewith 5 and imperfect contact results in high contact resistance and reduction in the output and efficiency of the thermo-couple.

Thermo-couples embodying the hereinbefore described members joined together by the hereinbefore described process have very little contact resistance at the joints in addition to the inherent ohmic resistance of the two elements. The thermo-couples have a long and useful life

and a high electrical output and their joints are not impaired when heated to a degree of 380° C. or even higher.

What I claim is:

1. A negative thermo-electric element alloy 80 consisting of 60 to 63% antimony, 1 to 4.5% arsenic and 34 to 37% zinc.

2. A thermo-couple, the positive element of which consists of an alloy of 55% copper and 45% nickel and the negative element of an alloy of 60-63% antimony, 34-37% zinc and 1-4.5% arsenic. 85

OTTO HERMANN.

15

90

20

95

25

100

30

105

35

110

40

115

45

120

50

125

55

130

60

135

65

140

70

145

75

150